

Nov. 22, 1949

A. F. THIEUZARD

2,488,837

PROCESS OF PRODUCING THREE-COLOR PHOTOGRAPHS

Filed April 26, 1946



Inventor  
Albert F. Thieuizard

By *J. J. Juvine*  
Atty.

## UNITED STATES PATENT OFFICE

2,488,837

## PROCESS OF PRODUCING THREE-COLOR PHOTOGRAPHS

Albert François Thieuzard, Paris, France

Application April 26, 1946, Serial No. 665,313  
In France January 30, 1946

1 Claim. (Cl. 95—2)

1

A process of producing three colour films, described in U. S. A. Patent No. 2,008,457 consists in applying two colours on both faces of films provided with two sensitive layers in using basic colourings, and to superimpose the third colour in using acid colouring on one face of the films after having resensitised the gelatine by means of potassium bichromate.

Above mentioned patent describes specially the addition of the red or yellow colours on the face bearing already the blue image. But it has been found that some of the specific colourings, though they allow to arrive at the wanted result, require careful handling in the preparation of coloured films, which renders very hazardous an industrial production. For instance, the specified red colouring (S rhodamine) is not firmly fixed by the mordant and the image becomes impaired if washing lasts too long a time. On another hand, the yellow colourings (F yellow, Mikado yellow, Thiazol yellow) penetrate slowly into the gelatine layer, which requires that they remain a long time in contact with this latter.

The object of the present invention is an improvement to the above mentioned process which will considerably facilitate the industrial production of three colour films.

The improved process is similar to the process described in the above-noted patent; it makes use of a film covered on both faces with a layer of gelatino silver bromide. After exposure under two monochrome negatives of the blue and red,

5 mate process. It has been found that Capri blue (tetramethyl-benzotoluoxazine chlorhydrate) and 5-B Rhoduline blue made by the Farbwerke of Hochst-on-the-Main, Germany (chemical name not known) are suitable for this purpose.

One face of the film bearing the two coloured images is then resensitized by impregnating the gelatine with an alkali bichromate and it is exposed under the monochrome positive of the third colour, yellow. The gelatine becomes insoluble at all places corresponding to the clear parts of the positive and more or less soluble at all places corresponding to the dark parts.

10 After washing, a yellow colouring is applied on the gelatine; it is more or less absorbed according to the solubility of the gelatine and a yellow image is thus added.

15 It has been found that none of the presently known yellow dyestuffs is entirely satisfactory. In fact the colourings for the yellow image must possess following properties:

20 1st—Color corresponding exactly to necessities of the three colour synthesis.

25 2nd—Quick penetration into the gelatine layer.

30 3rd—Dyeing in inverse proportion of the insolubility of the gelatine, white parts of the image being reserved.

4th—Good solubility at normal temperature.

35 New colourings have been found which meet all requirements. They are obtained by the copulation of aminopolysulphonic acids of naphthalene or benzene with diacetoacetic tolidide



40 The general formula of these colourings is as follows:



45 in which R is a benzene or naphthalene amine bearing a certain number of sulphonic groups so that the total number of these groups is 5 or 6.

50 The preparation of such a colouring is done for instance in the following manner:

A solution containing—

Water, 1 liter

55 Caustic soda, 120 grams or sodium carbonate, 160 grams

the film is developed and fixed and two silver images corresponding to blue and red selection positives are obtained. The silver images are then by a well-known process converted into images which will mordant basic dyes and they are dyed respectively in blue and red by means of basic dyestuffs.

The red image is obtained by means of red colourings derived from triphenylmethane known under the name of fuchsines. These colourings are firmly fixed by the mordant in definite quantity, namely in proportion with the amount of silver forming the image. The excess of colouring is removed by washing and the red image does not grow weak even if the washing is prolonged. The blue image is obtained by means of a basic dye which will not have any subsequent action during the preparation of the image by the bichro-

3

Naphthylamine 3.6.8. trisulphonic 1 acid, 383  
grams  
Sodium nitrite, 70 grams.

is cooled to 5° C. with ice, and poured out slowly into a cooled vessel containing:

Water, 1 liter  
Hydrochloric acid, 225 grams

The azo derivative precipitates; agitate so as to obtain a pulp at a temperature of about  $10^{\circ}$  C. Add slowly this pulp into a solution at a temperature of  $10^{\circ}$  to  $15^{\circ}$  C. containing:

Water, 1 liter  
Diacetoacetic tolidide, 190 grams  
Caustic soda, 40 grams  
Sodium carbonate, 10 grams

The colouring is formed quickly. Neutralize if necessary with hydrochloric acid. The solution may be diluted to a determined volume or evaporated for getting the dry colouring mixed with sodium chloride.

This new colouring penetrates quickly into the gelatine layer which reduces the time for producing films and it allows to superimpose the yellow either on the blue or the red image.

The replacement of the colourings previously used by the new ones facilitates the industrial production of three colour films in reducing the time of treatment and in keeping the exact balance of the colours as it corresponds to the basic silver images.

The accompanying drawing indicates the course of the coloring process according to the invention by a briefed flow diagram.

I claim:

A process for the production of photographic and cinematographic films in three colors from component monochrome negatives each taken

4

through an appropriate color screen, consisting in exposing the two faces of a film covered on both faces with a gelatino silver bromide emulsion respectively under two monochrome negatives 5 representing the blue and the red, developing, fixing and converting the silver images into images which will mordant basic dyes, dyeing both images respectively in blue and red by basic dyes, the dyestuff for the red being a fuchsine dye, 10 resensitizing one face of the film by bichromate, exposing it under a positive monochrome of the yellow and dyeing with a pinatype dyestuff of the formula



20 in which R is selected from the group consisting of benzene and naphthalene amines bearing not less than 5 and not more than 6 sulphonate groups.

ALBERT FRANÇOIS THIEUZARD.

#### REFERENCES CITED

The following references are of record in the file of this patent:

UNITED STATES PATENTS

| Number    | Name          | Date           |
|-----------|---------------|----------------|
| 1,278,667 | Ives          | Sept. 10, 1918 |
| 2,008,457 | Lessertisseur | July 16, 1935  |
| 2,210,905 | Eggert et al. | Aug. 13, 1940  |

## FOREIGN PATENTS

Number                   Country                   Date  
370,999           Great Britain ----- Apr. 18, 1932